

## UNITED STATES PATENT OFFICE

HAROLD R. RAFTON, OF LAWRENCE, MASSACHUSETTS, ASSIGNOR TO RAFFOLD PROCESS CORPORATION, A CORPORATION OF MASSACHUSETTS

## MANUFACTURE OF PAPER

No Drawing. Application filed April 8, 1929, Serial No. 353,667. Renewed July 28, 1931.

My invention relates to the manufacture of substantially unsized paper filled with alkaline filler.

The principal object of my invention is the improvement of machine operation in the manufacture of such paper.

An important object is the reduction, elimination, prevention or alteration of foam in such manufacture.

10 A further object is the improvement of machine operation particularly as regards dandy operation.

15 A further object is the diminution or substantial elimination of lumps, particularly wet end soft lumps, which tend to cause breaks on the machine.

A further object is the production of paper of a higher quality.

20 A further object is the production of paper of a more uniform quality.

A further object is the introduction of a small amount of breakable paraffin emulsion which may be precipitated if desired in the beater.

25 Other objects and advantages of my invention will become apparent during the course of the following description.

In my copending applications Serial Nos. 304,171 and 304,174 filed September 5, 1928, and No. 321,753, filed November 24, 1928, I have disclosed methods for the prevention of foam in substantially unsized paper filled with alkaline filler. Likewise in my copending application Serial No. 321,754, filed November 24, 1928, I have disclosed a method for the prevention of foam in either sized or substantially unsized paper; and in my copending applications Serial Nos. 325,407 and 325,408 both filed December 11, 1928, I have disclosed methods for the reduction or elimination of lumps in either sized or substantially unsized paper.

In said applications the methods disclosed were such that intimacy and/or time of contact between the alkaline filler and the alum

or the alum-sodium resinate or the like precipitate was substantially limited; or if the intimacy and/or time of contact had already resulted in deteriorating the effect of the alum or the alum precipitate, this effect was 50 subsequently restored under conditions where the intimacy and/or time of contact with the alkaline filler was substantially limited.

In my copending application Serial No. 262,030, filed March 15, 1928, I have disclosed 55 a method for sizing paper filled with alkaline filler in the beater wherein a paraffin emulsion is employed and flocculated—i. e. broken—by alkaline filler, and wherein in one variation thereof alum is employed thereafter. 60

I have now discovered a modification of that process wherein a breakable paraffin emulsion, such for instance as a saponaceous paraffin emulsion (i. e. a paraffin emulsion made with a saponaceous emulsifying agent) is thrown down—i. e. broken—by the action of an acidic precipitant such as alum instead of by alkaline filler.

I have found that the precipitate produced by an acidic precipitant such as alum 70 with a breakable paraffin emulsion, which for example in the case of a saponaceous paraffin emulsion may be considered to be an aluminum soap associated with paraffin, may be used in sizing paper filled with alkaline 75 filler as the precipitate is affected only very slowly by the action of alkaline filler, in fact so slowly that in the lengths of time ordinarily employed, it is not ordinarily affected thereby sufficiently to interfere with its practical use.

In my present invention, however, I am not concerned with sized paper, but with substantially unsized paper. Hence I employ in the manufacture of my paper breakable paraffin emulsions such as saponaceous paraffin emulsion, only in such an amount that, when it is thrown down by an acidic precipitant such as alum, it is insufficient to impart a substantial degree of sizing to the

paper, but is nevertheless beneficial in permitting the manufacture of the resulting unsized paper with a substantial diminution of lumps and foam, it not indeed to render 5 its manufacture substantially lump and foam free.

In the preferred practice of my invention I add to the fibrous material in the beater or like machine a suitable amount of breakable paraffin emulsion, for example saponaceous paraffin emulsion, allow a sufficient time for mixing, and then add a quantity of alum at least sufficient to completely throw down the said emulsion, although usually considerably more will be added owing to the relatively small amount of paraffin emulsion used. I then add alkaline filler. If the alkaline filler be added prior to the addition of the saponaceous paraffin emulsion and/or the alum, this will result in a prior flocculation of the emulsion by the alkaline filler as described in my above last referred to prior application. This latter procedure seems to require in certain cases a somewhat greater amount of emulsion to produce the same effect, so I preferably introduce the alkaline filler after the precipitation of the emulsion by the alum has taken place. Of course this is not always feasible especially when broke containing alkaline filler is used in the furnish, but in such case such broke may be added if desired prior to addition of the alum, and the remainder of the alkaline filler subsequent thereto. There is described below in this specification a suitable procedure which may be employed in this case. Coloring matter or other material may also be added as is customary in the beater.

After sufficient treatment in the beater, 40 the mix may be passed through the subsequent chests and treating apparatus, up to the point where it is diluted preparatory to introduction to the web-forming device of the paper machine. It is then diluted, 45 formed into a web, and passed through the usual drying and finishing machinery of the paper machine. The resulting paper may be further finished by the customary auxiliary machines, such as supercalenders if desired.

The addition of this small amount of emulsion has beneficial effects on machine operation, reducing or eliminating foam, reducing or preventing the filling up of the dandy 50 if a Fourdrinier machine be used, reducing or preventing the formation of soft lumps, particularly wet end soft lumps, thus reducing or eliminating breaks during machine operation. The quality and uniformity of the paper is thus improved.

While my invention may be practiced with any of the customary fibrous materials, such as mechanical and/or chemical pulps, it is particularly beneficial when used with furnishes containing old paper stock.

60 My invention is applicable to any grade

of substantially unsized paper made with an alkaline filler, and is especially advantageous when used in the manufacture of magazine paper, which may be supercalendered if desired, as this paper is run at relatively 70 high speeds in large tonnages, is sold in a highly competitive market, and any invention tending to better machine conditions during its manufacture is of great value.

The breakable paraffin emulsions that I 75 employ may be defined as emulsions breakable—i. e. precipitable—by the addition of an acidic material, such for example as alum. One example of such an emulsion is paraffin dispersed in an aqueous dispersion agent such 80 as in a solution of sodium silicate, and made in a known manner. The precipitate produced by alum in such case can be considered to consist substantially of aluminum silicate 85 associated with paraffin, which is affected by the action of alkaline filler only very slowly, so slowly in fact that in the lengths of time ordinarily employed, it is not ordinarily affected thereby sufficiently to interfere with its practical use, and it is thus incorporated 90 into the finished paper substantially unchanged. In such an emulsion as described above, it may be desirable at times to incorporate other materials in association with the paraffin as the disperse phase, such as 95 rosin, Montan wax or the like.

Another example of a breakable paraffin emulsion is a saponaceous paraffin emulsion. As explained above the precipitate produced by alum may in this case be considered to be 100 an aluminum soap associated with paraffin. The saponaceous paraffin emulsions which I have found suitable may be made with a variety of saponaceous emulsifying agents, e. g. sodium stearate, rosin size, or the like. 105 However, while I do not restrict myself thereto, I prefer to use rosin size as the emulsifying agent, because it is practically the cheapest of the light colored saponifiable materials. However at times a mixture of saponifiable materials may be used to advantage, for example rosin and Montan wax, the latter preferably in a minor percentage. Moreover those saponaceous emulsions in 110 which a relatively large proportion of emulsifying agent is employed are relatively more stable and less likely to deposit paraffin which may be a source of trouble at times, hence it is preferable to employ saponaceous emulsions in which the proportion of the emulsifying agent used is relatively large.

The saponaceous paraffin emulsions which I employ may be made in a variety of known ways, as for example in a machine suitable for intimate mixing, such as a colloid mill, homogenizer or the like. A suitable method is to melt together the saponifiable material, such as the rosin, with the paraffin, and then intimately mix the fluxed mass with an aqueous solution of an alkaline material, par- 130

ticularly a compound or compounds of an alkali metal, such for example as sodium. One suitable compound is sodium silicate; another is sodium hydroxide. If a colloid mill is to be used, proportionate quantities of the heated melt and the preferably heated alkaline solution, preferably in continuous streams, are directed into the orifice of the mill, from the exit of which issues the finished emulsion.

5 The action of the alkaline material is to saponify or partially saponify the saponifiable material such as the rosin, and the paraffin is emulsified probably simultaneously. The rosin exists in the emulsion in the form 10 of rosin size. When sodium hydroxide is used as the alkaline material a suitable amount has been found to be about seven per cent. of sodium hydroxide by weight based on the total weight of paraffin and rosin used.

15 Although this percentage has been found to hold approximately correct even for a considerable variation in the relative proportions of rosin and paraffin present, I do not restrict myself thereto as it may be widely varied. The concentration of the alkaline 20 solution may be such that the final emulsion issuing from the colloid mill may have as in one case found satisfactory, a concentration of 30 per cent. solids, although this percentage may vary widely and is in no sense 25 restrictive. The proportion of saponifiable material such as rosin to paraffin is subject to wide variation and I therefore do not restrict myself to any definite proportions.

30 However I have found, for example, that a 30 parts paraffin-70 parts rosin emulsion works satisfactorily, as does also an 18 parts paraffin-82 parts rosin.

The above examples are illustrative only 35 and not restrictive. Nor do I restrict myself to the above method of processing the emulsion as it will be understood by one skilled in the art that any other known method producing a substantially equivalent emulsion 40 will be suitable.

In regard to the flocculation or breaking of a saponaceous paraffin emulsion by alkaline filler, I have found that the emulsions which contain only substantially sufficient saponaceous 45 emulsifying agent to emulsify the paraffin are in general more sensitive to breaking by alkaline filler than those emulsions containing a large excess of saponaceous emulsifying agent. The emulsions, particularly of the latter group, although relatively less sensitive than the former, appear to have their sensitivity increased with increase of dilution. I have found that this sensitivity in dilute solution can be considerably reduced 50 by the addition of an alkaline material, for example sodium hydroxide, and this provides a method whereby in some cases, alkaline filler or broke containing same may be added to a beater in contact with a saponaceous paraffin 55 emulsion prior to the alum, and the floccula-

tion of the emulsion by said alkaline filler prior to the addition of the alum may be inhibited if not entirely prevented by the presence of sufficient alkali.

An illustrative formula suitable for practicing my invention is as follows:

|                                                                               | Pounds |
|-------------------------------------------------------------------------------|--------|
| Fibrous material (e. g. half sulphite and half soda pulp, air dry basis)---   | 1550   |
| Breakable paraffin emulsion e. g. saponaceous paraffin emulsion (dry basis) - | 20     |
| Alum                                                                          | 30     |
| Alkaline filler (e. g. calcium carbonate magnesium hydroxide, dry basis)---   | 450    |

Another illustrative formula is:

|                                                                                                           | Pounds |
|-----------------------------------------------------------------------------------------------------------|--------|
| Fibrous material (e. g. equal parts of sulphite pulp, soda pulp, and old paper stock, air dry basis)----- | 1600   |
| Breakable paraffin emulsion e. g. saponaceous paraffin emulsion (dry basis) -----                         | 85     |
| Alum                                                                                                      | 20     |
| Alkaline filler (e. g. calcium carbonate magnesium hydroxide, dry basis) ---                              | 400    |

The paraffin emulsion referred to in the above formulæ is a 70 parts rosin-30 parts paraffin emulsion, and in this instance 1 per cent. on the combined weight of fibre and filler is employed. As is well known to one skilled in the art, it takes, in general, more size to size a highly filled sheet than one of lower filler content. Moreover the degree of sizing obtained with any given furnish will depend to a considerable extent on the character of the stock, the degree of hydration, speed of the machine, and other known variables. Furthermore machines equipped with efficient white water recovery systems will give a sheet of higher filler content for any given filler content of the furnish than will one not so equipped, and this will effect the degree of sizing obtained. Hence it may be that in some cases an appreciable degree of sizing would be imparted by one per cent. of paraffin emulsion, whereas in others a substantially unsized sheet would be obtained.

These known variations must be taken into consideration in using the above formulæ, and if it should be found that in any given instance the conditions are such that the amount of emulsion recommended imparts to the sheet a substantial degree of sizing, the amount used should be cut down until a substantially unsized sheet is produced. Conversely in certain cases the amount of emulsion recommended may have to be increased, care being taken however not to go beyond the point where a substantially unsized paper is produced. Also in some cases it may be found that an amount of emulsion even less than that amount which is just insufficient to produce a substantial degree of

sizing in the paper will have a decidedly beneficial effect on machine operation, and in such cases it may be uneconomical to use more.

- 5 There may be certain cases in the practice of my invention where conditions will be such as to cause a certain deterioration of the alum-emulsion precipitate by the alkaline filler, such for instance as would be the case 10 if the time and/or intimacy of contact with the alkaline filler were excessive. In such cases it may be desirable to use extra alum added to the mix at or subsequent to its point of dilution prior to delivery to the web-forming device of the paper machine, in other words, at the wet end of the paper machine. In some cases where coated broke is employed this practice may aid in suppression of foam. In some cases even where no apparent deterioration 15 of the alum-emulsion precipitate has occurred, this practice may appreciably improve the effect of the alum-emulsion precipitate. Or it may be desirable to introduce the alkaline filler at the wet end of the 20 paper machine, either in whole or in part, and of course both of these practices can be combined, if desired, namely the alkaline filler (either in whole or in part) and the alum (either in whole or in part) may both 25 be added at the wet end of the paper machine, in this latter case the alum being preferably added prior to the alkaline filler.

Another variation is when the emulsion 30 preferably in dilute form may itself be added 35 to the fibrous material at the wet end of the paper machine, either alone or together with the alkaline filler (preferably followed thereby) and/or the alum, the alum being added 40 preferably before the alkaline filler; or the emulsion may be added in the beater and all 45 the alum at the wet end of the paper machine, in which case the alkaline filler may be added preferably at the wet end of the paper machine 50 preferably after the addition of the alum. Of course any addition to the mix at the wet end of the paper machine should be made preferably proportionately and preferably continuously, preferably in such a manner as to allow independent incorporation 55 of each individual ingredient with the mix, providing more than one ingredient is added.

I have found that in place of alum as a 60 precipitant for the emulsion, I may use with a certain measure of success certain acidic materials such as sulphuric acid ( $H_2SO_4$ ) or acid salts such as sodium bisulphate ( $NaHSO_4$ ), or other salts of aluminum, as the chloride or the like, or the double salts 65 which are the true alums; but because of its economy and of its general efficiency, I prefer to use the ordinary sulphate of aluminum, commonly called "alum". Any of the ordinary grades of alum, such as normal or 70 basic, may be used satisfactorily.

By the term "alkaline filler" I mean filler which when agitated in contact with freshly boiled distilled water, say for an hour, will impart a pH value to such water greater than 7.0, that is, which will be on the alkaline side of the neutral point. Among fillers included in this group may be mentioned calcium carbonate, of which lime mud from the causticizing process is one form; calcium carbonate magnesium basic carbonate employed in the paper disclosed in my United States Patent No. 1,595,416, issued August 10, 1926; calcium carbonate magnesium hydroxide disclosed in my United States Patent No. 1,415,391, issued May 9, 1922, and other substantially water insoluble normal or basic carbonates of alkaline earth metals, (which expression is herein intended to include magnesium), or compounds, double salts, or physically associated mixtures of these with one or more other acid soluble materials of a substantially water insoluble nature. It should be stated that any given filler of the type referred to is not necessarily of uniform particle size; nor are the average particle sizes 85 of the fillers necessarily alike, as some of the fillers of the type referred to have relatively coarse grain particles, whereas others are much more finely divided, and some are so finely divided that they may be said to approach or be in the colloidal condition. 90

By the term "alkaline filler" I also intend to include fibrous material and/or other material such as paper coating constituents or the like containing one or more compounds 100 of the character referred to, such as "old papers" or similar papers, "broke", or the like.

By the term "old paper stock", I mean to include deinked papers, either bleached or 105 not as desired, such as are commonly used for example in book and magazine paper furnishes. This material may contain filler such for example as clay which of course would vary in amount with the source and kind of old papers deinked and the particular modification of the deinking process used.

By the word "paraffin" I mean paraffin wax, which is solid at ordinary or room temperature. I do not restrict myself only to the 115 paraffin hydrocarbons, but mean to include in this word all the hydrocarbons of a waxy nature substantially unsaponifiable and inert to acidic and alkaline materials under ordinary conditions of temperature and pressure, 120 whether derived from petroleum, shale, lignite, earth wax, or other natural or artificial sources. I do not, however, mean to include in this term material of a pitchy nature.

When I use the word "paper" herein, I use it in the broad sense to include products of manufacture of all types and of all weights and thicknesses, which contain as an essential constituent a considerable amount of pre- 130

pared fibre and which are capable of being produced on a Fourdrinier, cylinder, or other forming, or felting, or shaping, or molding machine.

5 By the term "wet end of the paper machine" I intend to include those instrumentalities employed in paper manufacture by which and/or in which a relatively concentrated paper mix is diluted, and treated, conveyed or fed up to the point of web-formation, such as the mixing box, regulating and proportioning devices, riffles, troughs, screens, head boxes, inlets, and the like, including also instrumentalities used in the white water cycle.

When I use the word "rosin", I mean to include not only the natural material, but also any synthetic resin acid or acids.

When I use the term "rosin size", I mean to include any material produced by the action of an alkaline substance, generally in aqueous solution, on rosin, regardless of the exact composition of the product, or the degree of saponification, or the varying composition which different samples may possess.

When I use the term "alkali metal", I mean to include the hypothetical alkali metal ammonium.

While I have described in detail the preferred practice of my process it is to be understood that the details of procedure, the proportions of ingredients, and arrangement of steps may be widely varied without departing from the spirit of the invention or the scope of the subjoined claims.

I claim:

1. The method of manufacturing substantially unsized paper filled with alkaline filler comprising mixing fibrous material, breakable paraffin emulsion in an amount insufficient to impart a substantial degree of sizing to the paper, an acidic precipitant for said emulsion, and alkaline filler, and thereafter making paper therefrom.

45 2. The method of manufacturing substantially unsized paper filled with alkaline filler comprising mixing fibrous material, breakable paraffin emulsion in an amount insufficient to impart a substantial degree of sizing to the paper, alum, and alkaline filler, and thereafter making paper therefrom.

3. The method of manufacturing substantially unsized paper filled with alkaline filler comprising mixing fibrous material, saponaceous paraffin emulsion in an amount insufficient to impart a substantial degree of sizing to the paper, an acidic precipitant for said emulsion, and alkaline filler, and thereafter making paper therefrom.

60 4. The method of manufacturing substantially unsized paper filled with alkaline filler comprising mixing fibrous material, saponaceous paraffin emulsion in an amount insufficient to impart a substantial degree of sizing to the paper, the emulsification of

said emulsion having been effected with the aid of alkaline material, an acidic precipitant for said emulsion, and alkaline filler, and thereafter making paper therefrom.

5. The method of manufacturing substantially unsized paper filled with alkaline filler comprising mixing fibrous material, saponaceous paraffin emulsion in an amount insufficient to impart a substantial degree of sizing to the paper, the emulsification of said emulsion having been effected with the aid of an alkaline compound of an alkali metal, an acidic precipitant for said emulsion, and alkaline filler, and thereafter making paper therefrom.

70 6. The method of manufacturing substantially unsized paper filled with alkaline filler comprising mixing fibrous material, saponaceous paraffin emulsion in an amount insufficient to impart a substantial degree of sizing to the paper, the emulsification of said emulsion having been effected with the aid of an alkaline compound of sodium, an acidic precipitant for said emulsion, and alkaline filler, and thereafter making paper therefrom.

75 7. The method of manufacturing substantially unsized paper filled with alkaline filler comprising mixing fibrous material, saponaceous paraffin emulsion in an amount insufficient to impart a substantial degree of sizing to the paper, the emulsification of said emulsion having been effected with the aid of sodium hydroxide, an acidic precipitant for said emulsion, and alkaline filler, and thereafter making paper therefrom.

90 8. The method of manufacturing substantially unsized paper filled with alkaline filler comprising mixing fibrous material, saponaceous paraffin emulsion in an amount insufficient to impart a substantial degree of sizing to the paper, alum, and alkaline filler, and thereafter making paper therefrom.

95 9. The method of manufacturing substantially unsized paper filled with alkaline filler comprising mixing fibrous material, rosin size-paraffin emulsion in an amount insufficient to impart a substantial degree of sizing to the paper, an acidic precipitant for said emulsion, and alkaline filler, and thereafter making paper therefrom.

100 10. The method of manufacturing substantially unsized paper filled with alkaline filler comprising mixing fibrous material, rosin size-paraffin emulsion in an amount insufficient to impart a substantial degree of sizing to the paper, alum, and alkaline filler, and thereafter making paper therefrom.

110 11. The method of manufacturing substantially unsized paper filled with alkaline filler comprising mixing fibrous material, saponaceous rosin-Montan wax-paraffin emulsion in an amount insufficient to impart a substantial degree of sizing to the paper, alum, and alkaline filler, and thereafter making paper therefrom.

12. The method of manufacturing substantially unsized paper filled with alkaline filler comprising mixing fibrous material comprising sulphite and soda pulps, saponaceous paraffin emulsion in an amount insufficient to impart a substantial degree of sizing to the paper, alum, and alkaline filler, and thereafter making paper therefrom.
13. The method of manufacturing substantially unsized paper filled with alkaline filler comprising mixing fibrous material comprising sulphite pulp soda pulp and old paper stock, saponaceous paraffin emulsion in an amount insufficient to impart a substantial degree of sizing to the paper, alum, and alkaline filler, and thereafter making paper therefrom.
14. The method of manufacturing substantially unsized paper filled with alkaline filler comprising mixing fibrous material, saponaceous paraffin emulsion in an amount insufficient to impart a substantial degree of sizing to the paper, alum, and alkaline filler comprising alkaline earth metal carbonate, and thereafter making paper therefrom.
15. The method of manufacturing substantially unsized paper filled with alkaline filler comprising mixing fibrous material, saponaceous paraffin emulsion in an amount insufficient to impart a substantial degree of sizing to the paper, alum, and alkaline filler comprising calcium carbonate, and thereafter making paper therefrom.
16. The method of manufacturing substantially unsized paper filled with alkaline filler comprising mixing fibrous material, saponaceous paraffin emulsion in an amount insufficient to impart a substantial degree of sizing to the paper, alum, and alkaline filler comprising calcium carbonate and magnesium compound, and thereafter making paper therefrom.
17. The method of manufacturing substantially unsized paper filled with alkaline filler comprising mixing fibrous material, saponaceous paraffin emulsion in an amount insufficient to impart a substantial degree of sizing to the paper, alum, and alkaline filler comprising calcium carbonate magnesium hydroxide, and thereafter making paper therefrom.
18. The method of manufacturing substantially unsized paper filled with alkaline filler comprising mixing in the beater fibrous material, saponaceous paraffin emulsion in an amount insufficient to impart a substantial degree of sizing to the paper, alum, and alkaline filler, and thereafter making paper therefrom.
19. The method of manufacturing substantially unsized paper filled with alkaline filler comprising mixing in the beater fibrous material, saponaceous paraffin emulsion in an amount insufficient to impart a substantial degree of sizing to the paper, alum, and al-
- kaline filler, and adding a substantial quantity of alum at the wet end of the paper machine, and thereafter making paper therefrom.
20. In a method of manufacturing substantially unsized paper filled with alkaline filler the step of precipitating with alum a breakable paraffin emulsion in an amount insufficient to impart a substantial degree of sizing to a paper made therewith.
21. A paper comprising fibrous material, alkaline filler, and the precipitate produced by the action of alum on breakable paraffin emulsion, said precipitate being present in an amount insufficient to impart a substantial degree of sizing to said paper.
22. A paper comprising fibrous material, alkaline filler, and the precipitate produced by the action of acidic material on saponaceous paraffin emulsion, said precipitate being present in an amount insufficient to impart a substantial degree of sizing to said paper.
23. A paper comprising fibrous material, alkaline filler, and the precipitate produced by the action of acidic material on rosin size-paraffin emulsion, said precipitate being present in an amount insufficient to impart a substantial degree of sizing to said paper.
24. A paper comprising fibrous material, alkaline filler, and the precipitate produced by the action of alum on rosin size-paraffin emulsion, said precipitate being present in an amount insufficient to impart a substantial degree of sizing to said paper.
25. A paper comprising fibrous material, alkaline filler, and the precipitate produced by the action of alum on saponaceous rosin-Montan wax-paraffin emulsion, said precipitate being present in an amount insufficient to impart a substantial degree of sizing to said paper.
26. A substantially unsized paper comprising fibrous material, alkaline filler, paraffin and the precipitate produced by the action of alum on rosin size said paraffin and said precipitate being present in insufficient amount to impart a substantial degree of sizing to said paper.
27. A magazine paper comprising fibrous material including old paper stock, alkaline filler, paraffin and the precipitate produced by the action of alum on rosin size, said paraffin and said precipitate being present in insufficient amount to impart a substantial degree of sizing to said paper.
28. A supercalendered magazine paper comprising fibrous material including old paper stock, alkaline filler, paraffin and the precipitate produced by the action of alum on rosin size, said paraffin and said precipitate being present in insufficient amount to impart a substantial degree of sizing to said paper.
29. The method of manufacturing substantially unsized paper filled with alkaline

- filler comprising mixing fibrous material, breakable paraffin emulsion in an amount insufficient to impart a substantial degree of sizing to the paper, and an acidic precipitant 5 for said emulsion, subsequently adding alkaline filler to the mix, and thereafter making paper therefrom.
30. The method of manufacturing substantially unsized paper filled with alkaline filler 10 comprising mixing fibrous material, breakable paraffin emulsion in an amount insufficient to impart a substantial degree of sizing to the paper, and alum, subsequently adding alkaline filler to the mix, and thereafter making 15 paper therefrom.
31. The method of manufacturing substantially unsized paper filled with alkaline filler comprising mixing fibrous material, saponaceous paraffin emulsion in an amount insufficient 20 to impart a substantial degree of sizing to the paper, and an acidic precipitant for said emulsion, subsequently adding alkaline filler to the mix, and thereafter making paper therefrom.
- 25 32. The method of manufacturing substantially unsized paper filled with alkaline filler comprising mixing fibrous material, saponaceous paraffin emulsion in an amount insufficient 30 to impart a substantial degree of sizing to the paper, the emulsification of the said emulsion having been effected with the aid of alkaline material, and an acidic precipitant for said emulsion, subsequently adding alkaline 35 filler to the mix, and thereafter making paper therefrom.
33. The method of manufacturing substantially unsized paper filled with alkaline filler comprising mixing fibrous material, saponaceous 40 paraffin emulsion in an amount insufficient to impart a substantial degree of sizing to the paper, the emulsification of said emulsion having been effected with the aid of an alkaline compound of an alkali metal, and an acidic precipitant for said emulsion, subsequently 45 adding alkaline filler to the mix, and thereafter making paper therefrom.
34. The method of manufacturing substantially unsized paper filled with alkaline filler comprising mixing fibrous material, saponaceous 50 paraffin emulsion in an amount insufficient to impart a substantial degree of sizing to the paper, the emulsification of said emulsion having been effected with the aid of an alkaline compound of sodium, and an acidic 55 precipitant for said emulsion, subsequently adding alkaline filler to the mix, and thereafter making paper therefrom.
35. The method of manufacturing substantially unsized paper filled with alkaline filler comprising mixing fibrous material, saponaceous 60 paraffin emulsion in an amount insufficient to impart a substantial degree of sizing to the paper, the emulsification of said emulsion having been effected with the aid of sodium 65 hydroxide, and an acidic precipitant for said emulsion, subsequently adding alkaline 70 filler to the mix, and thereafter making paper therefrom.
36. The method of manufacturing substantially unsized paper filled with alkaline filler 75 comprising mixing fibrous material, saponaceous paraffin emulsion in an amount insufficient to impart a substantial degree of sizing to the paper, and alum, subsequently adding alkaline filler to the mix, and thereafter making 80 paper therefrom.
37. The method of manufacturing substantially unsized paper filled with alkaline filler comprising mixing fibrous material, rosin size-paraffin emulsion in an amount insufficient 85 to impart a substantial degree of sizing to the paper, and an acidic precipitant for said emulsion, subsequently adding alkaline filler to the mix, and thereafter making paper therefrom.
38. The method of manufacturing substantially unsized paper filled with alkaline filler comprising mixing fibrous material, rosin size-paraffin emulsion in an amount insufficient 90 to impart a substantial degree of sizing to the paper, and alum, subsequently adding alkaline filler to the mix, and thereafter making paper therefrom.
39. The method of manufacturing substantially unsized paper filled with alkaline filler comprising mixing fibrous material, saponaceous rosin-Montan wax-paraffin emulsion in an amount insufficient to impart a substantial 95 degree of sizing to the paper, and alum, subsequently adding alkaline filler to the mix, and thereafter making paper therefrom.
40. The method of manufacturing substantially unsized paper filled with alkaline filler comprising mixing fibrous material comprising sulphite and soda pulps, saponaceous 100 paraffin emulsion in an amount insufficient to impart a substantial degree of sizing to the paper, and alum, subsequently adding alkaline filler to the mix, and thereafter making 105 paper therefrom.
41. The method of manufacturing substantially unsized paper filled with alkaline filler comprising mixing fibrous material comprising sulphite pulp, soda pulp and old paper stock, saponaceous paraffin emulsion in an amount insufficient to impart a substantial 110 degree of sizing to the paper, and alum, subsequently adding alkaline filler to the mix, and thereafter making paper therefrom.
42. The method of manufacturing substantially unsized paper filled with alkaline filler comprising mixing fibrous material, saponaceous 115 paraffin emulsion in an amount insufficient to impart a substantial degree of sizing to the paper, and alum, subsequently adding to the mix alkaline filler comprising alkaline earth metal carbonate, and thereafter making paper therefrom.
43. The method of manufacturing substantially unsized paper filled with alkaline filler 120 comprising mixing fibrous material, saponaceous paraffin emulsion in an amount insufficient to impart a substantial degree of sizing to the paper, and alum, subsequently adding to the mix alkaline earth metal carbonate, and thereafter making paper therefrom.

comprising mixing fibrous material, saponaceous paraffin emulsion in an amount insufficient to impart a substantial degree of sizing to the paper, and alum, subsequently adding 5 to the mix alkaline filler comprising calcium carbonate, and thereafter making paper therefrom.

44. The method of manufacturing substantially unsized paper filled with alkaline filler 10 comprising mixing fibrous material, saponaceous paraffin emulsion in an amount insufficient to impart a substantial degree of sizing to the paper, an alum, subsequently adding 15 to the mix alkaline filler comprising calcium carbonate and magnesium compound, and thereafter making paper therefrom.

45. The method of manufacturing substantially unsized paper filled with alkaline filler comprising mixing fibrous material, saponaceous 20 paraffin emulsion in an amount insufficient to impart a substantial degree of sizing to the paper, and alum, subsequently adding 25 to the mix alkaline filler comprising calcium carbonate magnesium hydroxide, and thereafter making paper therefrom.

46. The method of manufacturing substantially unsized paper filled with alkaline filler comprising mixing in the beater fibrous material, saponaceous paraffin emulsion in an amount insufficient to impart a substantial degree of sizing to the paper, and alum, subsequently adding alkaline filler to the mix, and thereafter making paper therefrom.

47. The method of manufacturing substantially unsized paper filled with alkaline filler comprising mixing in the beater fibrous material, saponaceous paraffin emulsion in an amount insufficient to impart a substantial degree of sizing to the paper, and alum, subsequently adding alkaline filler to the mix, adding a subsequent quantity of alum at the wet end of the paper machine, and thereafter making paper therefrom.

In testimony whereof I affix my signature.

HAROLD ROBERT RAFTON.